

# UNITED STATES PATENT OFFICE.

EDGAR ARTHUR ASHCROFT, OF LONDON, ENGLAND.

## ELECTROLYTIC PRODUCTION OF SODIUM ALLOYS.

1,161,585.

Specification of Letters Patent.

Patented Nov. 23, 1915.

No Drawing.

Application filed November 22, 1913. Serial No. 802,582.

To all whom it may concern:

Be it known that I, EDGAR ARTHUR ASHCROFT, a subject of the King of Great Britain, and residing at 99 Buckingham Palace road, London, England, and Plumley, Bovey Tracey, England, have invented new and useful Improvements in the Electrolytic Production of Sodium Alloys, of which the following is a specification.

It is known that it is possible to electrolyze molten alkali hydroxids, alkali metal and hydrogen being thereby formed at the cathode and oxygen at the anode, and it has been proposed to cause the alkali metal to be taken up at the cathode by molten heavy metal such for example as lead. It has also been proposed to use, in the arts, the alloys of the alkali metals with a heavy metal instead of using the pure metals. The electrolysis takes place as is known in accordance with the following formula:



The hypothetic radical hydroxyl reacts at once in accordance with the following formula:



and the water thus formed is at once absorbed by the melt. Before fresh alkali metal can form, energy for the decomposition of the water absorbed by the melt must be consumed, or what comes to the same thing, only 1 molecular proportion of sodium is formed out of 2 molecular proportions of sodium the second molecular proportion of sodium being consumed in decomposing the water formed at the anode and this reduction of the current efficiency to half that theoretically possible, is characteristic of all the processes in which caustic alkalis have been electrolyzed by means of insoluble anodes. For instance, in the Castner process described in the specification of German Patent No. 58121 the practical current efficiency is lower than 40 per cent. and the operation is carried out at a temperature of 350° centigrade. Castner says in his specification:

"In order to insure a suitable yield of alkali metal for the current supplied, it is necessary that the temperature of the electrolyte should not be allowed to exceed the melting point of the caustic alkali used by more than 20° centigrade, that is when treating caustic soda which melts at about 310° centigrade, the temperature of the electro-

lyte should be kept below 330° centigrade. The same should be observed for caustic potash, or a mixture of both hydroxids, which has a lower melting point than the caustic potash and caustic soda taken each by itself."

Lorenz describing a phenomenon of polarization has drawn attention to the influence of the temperature and of the voltage required for the decomposition (Lorenz, *Electrolysis of Molten Salts*, published by Knapp, Halle 1906, part 3, pages 278 and 279). Other experimenters have stated that, for the successful electrolysis of, for instance, caustic soda, the temperature must be below 400° centigrade.

While the above prescriptions for the production of pure sodium have hitherto not been contradicted, I have ascertained that, for the production of lead sodium the conditions are different and that by the use of a higher temperature the extra consumption of energy required for the decomposition of water can be avoided, partly, or wholly. According to my invention the water is partly, or wholly, expelled as such at a high temperature, so that mainly oxygen and aqueous steam escape from the electrolyzing vessel and not oxygen and hydrogen as in the hitherto known processes. For the more, or less, complete carrying out of my new process, I carry on the electrolysis at a temperature of, or over, 400° centigrade, and I observe the following important precautions, all of which tend to the production of a result as perfect as possible. Firstly that the layer of the alkali hydroxid above the heavy metal alloy, shall be comparatively thin; secondly, that both the electrolyte and the alloy shall be kept in motion, for instance by means of magnetic stirring, and thirdly, that the operation shall be carried out with a current density as high as possible at the anode. The alloys obtained can be used as such, or be further treated so as to obtain alkali metal, or alkali metal compounds, which latter can be done in a separate operation or in a secondary cell connected with the electrolyzing cell.

When a secondary cell is used, the operation can be conducted for example as follows: A cathode of molten heavy metal, for instance lead, with about from 6, to 12 per cent. of sodium is placed in a circular shallow flat cell provided with properly ar-

- ranged inlet and overflow pipes, and connected in one steel casting with a secondary cell and a collecting vessel as described in the specifications of British Letters 5 Patent Nos. 1001 to 1005 A. D. 1912 granted to me. Over the cathode is a thin layer of electrolyte which, together with the cathode metal, is kept at a temperature between 400° and 500° centigrade, while the alloy 10 in addition to being circulated in the apparatus by a pump (in accordance with the above named specifications), is rotated by a magnetic stirring device (see the specification of British Letters Patent No. 5648 A. D. 15 1905 granted to me). By these means the formation in the alloy, of layers of different specific gravities and of deposits on the surface of the cathode is avoided while the escape of the aqueous steam is promoted. 20 By working in this manner, yield efficiencies of current of from 60, to 80 per cent, and more, can be obtained. As in most processes of this kind the heat is produced by the electric current and regulated by a suitable selection 25 of the current density. The anode can be of nickel, or any other suitable metal, and is preferably so arranged that the current enters at a row of points distributed in a suitable manner over the area 30 of the cathode and connected with an annular plate.
- The apparatus which is described in the aforesaid specifications of my previous British Patents Nos. 1001 to 1005 A. D. 1912 35 is very suitable for the purpose in view if the earthenware lining be omitted and a lining of copper, nickel or other suitable metal be substituted and the graphite anode be replaced by the aforesaid annular anode 40 plate of nickel. The pipes for the escape of chlorin from the aforesaid apparatus are in the present process used for carrying away the spray of alkali which is entrained with the steam and would contaminate the air. 45 Such spray is condensed in a suitable condensation chamber. From time to time the dirt which has deposited in the cell must be removed, as this dirt would otherwise accumulate and disturb the course of the electrolysis. It is known that, for all such processes, apparatus as large as possible is of 50 importance for economical operation. The process herein described is especially suitable for the employment of large units. It is thus preferable to work a double cell apparatus with 10,000 amperes. If for instance, metallic sodium is produced in the secondary cell, a total voltage of about 5 volts is used, including of course, the heat energy required 55 for heating both cells. It is known that in the Castner process employed, especially for the production of sodium, only apparatus of about 1250 amperes, or thereabout have been used and that a large number of cells are required 60 to produce a given quantity of metal. 65

In the process herein described more than ten times such quantity of sodium can be readily manufactured. Not only is the labor required less, but the consumption of energy is also much less for a given quantity of product.

It is obvious that the hereinbefore described process can be used for the production of alkali-metal alloys without departing from the invention if such alloys are to 75 be used as final products for industrial purposes. It is however likewise obvious that the process can be used directly in combination with known methods for the production of valuable products such as alkali metals, amids, cyanamids, cyanids and the like, in the secondary cell attached to the said apparatus, with, or without, the use of the electrolysis as described for instance in the British specification No. 228 of A. D. 1910. 80 85

What I claim is:—

1. The process of producing alloys of sodium and heavier metals which consists in subjecting an electrolyte of molten sodium hydroxid to electrolysis between a suitable 90 anode and a cathode of a molten heavy metal, the electrolysis being carried out at a temperature of about 400° centigrade.

2. The process of producing alloys of sodium and heavier metals which consists in 95 subjecting an electrolyte of molten sodium hydroxid to electrolysis between a suitable anode and a cathode of a molten heavy metal, the electrolysis being effected at a temperature of at least substantially 400° 100 centigrade.

3. The process of producing alloys of sodium and heavier metals which consists in subjecting an electrolyte of molten sodium hydroxid to electrolysis between a suitable 105 anode and a cathode of a molten heavy metal, maintaining the sodium hydroxid in a thin layer on the cathode during electrolysis and effecting the electrolysis at a temperature of about 400° centigrade.

4. The process of producing alloys of sodium and heavier metals which consists in subjecting an electrolyte of molten sodium hydroxid to electrolysis between a suitable 110 anode and a cathode of a molten heavy metal at a temperature of about 400° centigrade while maintaining a high current density at the anode.

5. The process of producing alloys of sodium and heavier metals which consists in 115 subjecting an electrolyte of molten sodium hydroxid to electrolysis between a suitable anode and a cathode of a molten heavy metal at a temperature of about 400° centigrade, while maintaining the electrolyte and cathode metal in motion during electrolysis.

6. The process of producing alloys of sodium and heavier metals which consists in subjecting an electrolyte of molten sodium hydroxid to electrolysis between a suitable 120 125 130

anode and a cathode of a molten heavy metal, maintaining the electrolyte in a thin layer, while keeping the electrolyte and cathode in motion, the operation being effected with a high current density at the anode and at a temperature of about 400° centigrade.

In testimony whereof I have signed my name to this specification in the presence of two subscribing witnesses.

EDGAR ARTHUR ASHCROFT.

Witnesses:

WALTER WILLIAM EDGECOMBE,  
JOSEPH HENRY WILLS.